

# United States Patent Office.

BENJAMIN SILLIMAN, OF NEW HAVEN, CONNECTICUT.

*Letters Patent No. 95,941, dated October 19, 1869.*

## IMPROVEMENT IN THE MANUFACTURE OF ILLUMINATING-GAS.

The Schedule referred to in these Letters Patent and making part of the same

*To all whom it may concern:*

Be it known that I, BENJAMIN SILLIMAN, of the city of New Haven, in the county of New Haven, and State of Connecticut, have discovered a new and useful Material for the Manufacture or Production of Gas for Illuminating or Heating-Purposes; and I do hereby declare that the following is a full, clear, and exact description thereof, such as will enable those skilled in the art to use the same.

The material or substance is an extremely rich and entirely peculiar mineral hydrocarbon, and is found in the Wollongong district of the Illawara coal-field, in New South Wales, and is called by me by the name of Wollongongite.

Its mineralogical characters are as follows:

In cubical or oblong blocks, without lamination. Breaks with great difficulty, in broad conchoidal surfaces. Is extremely tough, and resounding like hard wood under the blows of the hammer. Hardness, from 2 to 2.5; and gravity, 1.04 to 1.5. Lustre, silky. Color, greenish black and brownish yellow; streak, light brown to yellowish. No odor when rasped. Tasteless. Sectile, thin shavings curling up under the knife. Not electric by friction of the mass, but shavings cut off by the knife are highly electric. Translucent in thin shavings; and these, under the microscope, transmit amber yellow light. Alone in a test-tube, does not melt nor swell up; decrepitates and exhales a light vapor, and distils a copious flow of oil, of a yellow color and heavy odor, giving off much gas. Is insoluble in alcohol, ether, or benzole, but is slightly acted on by carbonic disulphide or bisulphuret of carbon, to which it imparts a slightly yellow tinge. Chloroform dissolves from it a minute amount of a substance resembling wax or vegetable tallow. Is readily kindled in thin splints by a match, burning with a brilliant flame and much smoke.

From this description every person skilled in a knowledge of mineral characters will at once see that this substance is not a coal, but is much more like succinite or amber in some of its characters, while in others it recalls some of the attributes of the Torbane Hill mineral or Bog-head cannel, from which, however, it is separated by well-characterized qualities.

By a series of careful experiments I have discovered and demonstrated that this material or Wollongongite is by far the most remarkable mineral substance hitherto described or made known for the production of illuminating-gas, whether treated by

the ordinary gas-making process for obtaining gas from coal, or by the hydrocarbon process.

By the common process of the gas-house it yields about fourteen thousand cubic feet of gas to the ton of twenty-two hundred and forty pounds, having an illuminating-power or intensity of over one hundred and thirty candles, giving six cubic feet of gas per pound; one cubic foot of the gas being equal to the light of twenty-six sperm candles.

One ton of this material yields over eighteen hundred pounds of gas, and only about four hundred and twenty pounds of very light and lustrous carbon.

By the hydrocarbon process, this Wollongongite yields over fourteen cubic feet of gas per pound of the material. Its gas-producing power is such that a good sample of common caking coal, which alone gives only about ten thousand cubic feet of gas, of fourteen candles' power, will, when mingled with not over ten per cent. of the Wollongongite, yield over sixteen thousand cubic feet of gas to the ton of mixture, of an illuminating-power of over twenty candles.

These statistics are sufficient to show to all who are skilled in the art of gas-making that such researches of mine have contributed or made known to that art a material beyond comparison more valuable than any hitherto known among the various mineral hydro-carbons which are available for use in the gas-house.

I consider it preferable that this material should be employed in the hydrocarbon-gas process, as in that way it more fully develops its remarkable powers; but it may be used with great advantage in small quantities as an enriching material to enhance the value of caking coals.

If used by itself, the quantity of hydrocarbon or water-gases should be proportionately increased.

What is claimed, and desired to be secured by Letters Patent, is—

The use and application of the material or mineral hydrocarbon called Wollongongite, possessing the attributes and qualities substantially as above described, either by itself or mixed with other gas-producing substances, for the purpose of making gas for illuminating or heating-purposes.

B. SILLIMAN.

Witnesses:

S. D. LAW,  
F. E. VAN AUKEN.